

## UNITED STATES PATENT OFFICE

HENRY V. DUNHAM, OF BAINBRIDGE, NEW YORK

## GLUE AND METHOD FOR MAKING PLYWOOD

No Drawing.

Application filed September 24, 1929. Serial No. 394,925.

This invention has for its object the making of a glue or adhesive suitable for use in gluing together wood objects and the like and particularly wood veneers by processes known in the art and this adhesive is suitable for use where the so-called hot plate process is employed in which heat and pressure are used simultaneously in joining the several plies or parts to be joined. In the 10 hot plate process type of gluing the usual method is to dissolve dry blood or blood albumin in water and to apply this dissolved material to wood such as veneers for the purpose of making three-ply panels or other 15 multi-ply panels by applying the glue in the usual manner well known in the art of plywood manufacture. When the solution of blood or albumin has been applied to the veneers and the latter assembled to constitute the panels they are placed in hydraulic presses which are equipped with steam heated platens. As a general thing about 20 three glued up panels are placed between each set of platens and from 300 to 500 pounds 25 per square inch of pressure applied for from 3 to 5 minutes. The temperature of the heated platens may be about 250° F. or in some cases somewhat higher.

When pressed between hot plates in this 30 manner, the panels become heated up somewhat. Even when three three-ply panels are pressed between the two hot plates, the inner panel becomes hot enough to be uncomfortable to handle. During this treatment, 35 the glue joint becomes hot enough to coagulate the albumin and to set the glue. Perhaps steam generated in the hot pressing may assist in this.

By this procedure the glued panels obtained 40 have a good dry strength and due to the heat applied to the liquid blood there is a coagulation of the albumin to such an extent that the glued panels will not separate easily when soaked in water. Such types of glued 45 woods are employed in airplane construction and other commercial lines of manufacture where good water-resistance is desired.

There are, however, certain objections to 50 the use of blood albumin for this type of gluing. In the first place it is quite expen-

sive. It also lacks covering capacity when dissolved as compared with many other types of glues. It has a tendency toward great penetration into the wood and thus not leaving a sufficient film of glue on the wood surface, particularly on some types of soft woods such as poplar, pine, fir, and the like. 55

By my invention I have found that I can secure an improved blood albumin glue particularly suitable for hot plate press work, 60 which will remain usable longer than blood albumin, will have a better flow when applied to panels and the like, and will give a more uniform layer of film of glue on the glued surface. To obtain these results I mix 65 with the blood albumin the desired quantities of mixtures of finely ground seed meal and alkali or casein, alkali and a finely ground seed-meal containing a relatively 70 high percentage of protein.

In order to more fully describe and explain my invention I give herewith, examples by way of illustration, and tests showing several combinations which have proved to be 75 satisfactory although I do not limit myself to the examples and proportions cited.

In referring to blood or blood albumin I mean dried blood or what is known and sold commercially as dried blood albumin. Obviously the blood or blood albumin could be 80 used in the undried condition although this is not usually practical due to the rapid decomposition of the blood in this form.

In referring to casein, I mean a dried 85 milk casein of ordinary commercial grade, preferably ground to pass a 50 mesh standard wire screen or finer.

In referring to seed-meals I mean the meal from protein-rich seeds, such as the 90 peanut, cotton-seed, soy bean and the like, which have been finely ground preferably so that practically all of the meal will pass through an 80 mesh standard wire sieve and preferably a meal or flour made from the 95 press cake of the seed, after the major portion of the oil or fat has been extracted or removed by the usual commercial process employed in extracting or expressing the natural oil content of the seeds. These seed, 100

meals preferably contain about 3 to 6% of the natural oil content of the seeds.

In referring to alkalies I means water-soluble salts or compounds of alkali and/or 5 alkaline earths which when dissolved react alkaline to litmus paper such for example, as calcium hydrate, sodium phosphate, sodium carbonate, sodium fluoride, caustic soda and the like, or preferably mixtures of the 10 alkali metal compounds (sodium compounds) and alkaline earth compounds (slaked lime).

Referring now to specific examples:—

*Example 1*

15 90 parts of blood albumin, 30 parts of casein, 30 parts of peanut meal, 100 parts of sawdust. These ingredients are preferably mixed together dry and are added to 600 parts of cold water and slowly mixed for 20 from 20 minutes to half an hour. Then another 600 parts of cold water are added, the mass well mixed and allowed to stand for 1 hour. At the end of the hour I add 36 parts 25 of commercial hydrated lime previously mixed in 54 parts of water. I then mix for about five minutes, then add 5 parts of sodium silicate, mix another 5 minutes when the glue is ready to be used.

*Example 2*

30 90 parts of blood albumin, 15 parts of casein, 45 parts of peanut meal, 100 parts of sawdust, preferably mixed together dry and proceed as in Example 1.

*Example 3*

40 90 parts of blood albumin, 15 parts of casein, 45 parts of peanut meal, 5 parts of tri-sodium phosphate, 100 parts of sawdust, mixed together dry and proceed as in Example 1, (including the addition of lime and sodium silicate).

*Example 4*

45 90 parts blood albumin, 60 parts soybean meal, 5 parts tri-sodium phosphate, 2 parts sodium fluoride, 100 parts sawdust. Mix together dry and proceed as in Example 1.

I am of course aware that blood albumin 50 and alkalies have been used in adhesives, and make no claim thereto. Also casein and seed-meals have been used with alkali. But, as I have clearly demonstrated by actual tests, there is an unexpected coaction between the 55 constituents of this compound glue. To illustrate this, I cite an experiment made with the identical mixture of Example 1, above, but omitting the casein and peanut meal. The glue could be mixed exactly in accordance with that example. However within a few minutes after the completion of the mixing, the glue became so thick as to be no longer spreadable by an ordinary glue spreading machine. With the casein and peanut meal added, as per Example 1, the

glue was spreadable upon the glue machine for about two hours.

Stated otherwise, the glue made from blood albumin, sawdust, lime, sodium silicate and water would be impractical since it has a "life" of only a few minutes, whereas when the casein and peanut meal are added, the "life" is about two hours. This first would be impractical for use on a spreading machine, whereas the later would be practical.

With the glues prepared as per Examples 2 and 3, above, the "life" will vary between 1.5 and 3 hours, more or less, depending on proportions, etc. With Example 4, a still thinner glue is formed, suitable for some types of plywood, which does not thicken for a longer time than the other examples above.

Obviously other combinations of these ingredients may be made and varying proportions employed depending upon the type of wood that is to be glued and other features well known in the art of the gluing of wood.

In the above formulas, I can use other alkaline salts of alkali metals (say sodium carbonate, di-sodium phosphate, etc.) in place of the tri-sodium phosphate. In using caustic soda, this will ordinarily be added to the water used in making up the liquid glue, or it can be added with the lime. The lime and sodium salts would seem to react on mixing with water.

The sawdust used can be hardwood or soft-wood sawdust, preferably ground to pass a 40 mesh screen, or finer. It might be as fine as the seedmeal or flour, or finer. Equivalent materials such as corn cobs, chaff from grain, hulls from seeds, ground peanut shells, or the like, can be substituted. Sawdust and equivalent material will hereinafter be included in the term "cellulosic material".

For securing the strongest joints I prefer to use some casein at least in the formula. Even a small amount improves the product somewhat. Where very soft woods are employed and only relatively waterproof results are desired and where cost is an important factor, I may use a formula without the casein being used. The casein and lime used together assist in giving good waterproof joints.

It will be understood that all or a part only of the ingredients of the final glue can be made up by the glue manufacturer and the other materials added, say at the time of making up the liquid glue.

For instance the blood albumin, casein, and seed-meal, with or without sawdust, could be made and sold by the glue manufacturer, with instructions on the package as to adding the other components, to be added by the user. Likewise the casein and seed-meal, with or without the dry lime hydrate and sodium salts and/or blood albumin, could be

sold by the glue manufacturer, all as well known in the dry glue industry.

It will be understood that glues of this type are generally sold in the dry state, and only 5 mixed with water to form the liquid glue at the time of use or a few hours, at the most, before use.

The method of applying the glues illustratively given in the above examples is the same 10 as when applying any other glue, as by means of glue rolls or by spreading the glue on the wood with a brush or by any other desired manner, putting the glued panels in the hydraulic press between the heated platens, applying 15 desired pressure and temperature for a period usually not exceeding 5 minutes, then the panels may be removed, stacked for drying for a few days if desired when they are ready to be used as required.

20 By following this disclosure I have been able to secure glued wood of a veneer panel type which has shown dry strengths on the Riehle testing machine, (which is a standard testing machine for testing plywood 25 strengths) of as high as 430 pounds per square inch for the dry strengths and samples of this type of glued wood when soaked in water for 48 hours show no separation even at the edges of the specimen samples and have 30 shown as high as 270 pounds wet strength per square inch after this 48 hour soaking period.

While I have particularly described the application of the glue of this invention in the hot plate process, in which the present glue is 35 very suitable, it is to be understood that the glue described is not limited to use in this process.

I claim:—

1. A glue base comprising as its essential 40 constituents blood albumin, seed-meal rich in protein, and casein, which base upon mixing with water, alkali and an alkaline earth can produce a glue suitable for making waterproof plywood.

45 2. A glue base comprising blood albumin, seed-meal rich in protein, and casein, and cellulosic material, which base upon mixing with water, alkali and an alkaline earth can produce a glue suitable for making waterproof plywood.

50 3. A glue comprising as its essential constituents the reaction products of blood albumin, seed-meal of high protein content, alkali and water, such glue being substantially free from added rubber and from formaldehyde material.

55 4. A glue comprising as its essential constituents the reaction products of blood albumin, seed-meal of high protein content, 60 casein, lime, alkali and water.

5. A glue comprising the reaction products 65 of blood albumin, seed-meal of high protein content, cellulosic material, alkali and water, such glue being free from rubber and from 70 formaldehyde and its compounds.

6. A glue base comprising blood albumin, seed-meal rich in protein, and casein, and an amount of comminuted cellulosic material greater than any one of said named materials, which base upon mixing with water, alkali and an alkaline earth can produce a glue 75 suitable for making waterproof plywood.

7. A glue comprising the reaction products of blood albumin, seed-meal of high protein content and a comminuted cellulosic material greater than any one of said named materials, alkali and water.

8. A glue comprising the reaction products of blood albumin, seed-meal of high protein content, casein, lime, alkali and water, and a comminuted cellulosic material constituting the largest solid ingredient.

9. A glue comprising the reaction products of blood albumin, seed-meal of high protein content, casein, lime, alkali and water, said 85 glue having a "life" several times greater than the "life" of a glue with the corresponding proportion of blood albumin, lime and alkali, but without the casein and seed meal added.

10. A glue comprising the reaction products of blood albumin, seed-meal of high protein content, cellulosic material, said cellulosic material being in amount greater than any of 90 said mentioned material, alkali and water.

11. A glue base comprising 90 parts of dried blood albumin, 15 to 30 parts of dried milk casein, 30 to 45 parts of highly proteinaceous seed meal and about 100 parts of fine comminuted cellulose, such base when mixed with water and alkalies producing a smooth glue having a "life" much longer than the life of 100 a similar glue without the casein and seed meal.

In testimony whereof I affix my signature. 105  
HENRY V. DUNHAM.

110

115

120

125

130